

# UNITED STATES PATENT OFFICE.

MOVSESS B. ADOM, OF WHITE PLAINS, NEW YORK.

## PROCESS OF RENDERING TEXTILE FABRICS ANTIQUE.

1,227,361.

Specification of Letters Patent.

Patented May 22, 1917.

No Drawing.

Application filed June 28, 1915. Serial No. 36,750.

To all whom it may concern:

Be it known that I, MOVSESS B. ADOM, a citizen of the United States, and a resident of White Plains, county of Westchester, 5 and State of New York, have invented a new and Improved Process of Rendering Textile Fabrics Antique, of which the following is a full, clear, and exact description.

My invention relates to a process for rendering textile fabric antique, and it has reference particularly to the process for rendering tapestry antique, and more particularly oriental rugs.

The object of the invention is to provide 15 a simple, inexpensive, rapid and efficient process whereby newly manufactured textile fabrics can be rendered antique by reducing the brightness of the colors and giving a luster to the fabric. The ordinary process employed at present is very slow, as the reducing of different colors, whether anilin or vegetable, or both, is done in successive steps requiring a great deal of time and care.

25 With my process the subduing of the colors, no matter of what nature, is obtained by means of a single bath in which the reduction of the colors is obtained, while the whites of the fabric are prevented from being discolored. The textile fabric to be rendered antique, that is, the colors of which are to be subdued, is treated as follows:

After the preliminary cleaning, the fabric is immersed in a bath containing the following ingredients, having the following proportions by weight: caustic soda, 1 per cent.; and sodium bisulfite, 4 per cent. The bath is at about 100 degrees Fahrenheit, which temperature is gradually raised to 40 substantially 140° F. It may be remarked that the percentage of ingredients in the bath and the temperature thereof will vary according to the quality and grade of carpet, or other fabric, and the nature of the dye stuff thereon; that is to say, whether the dyes are anilin or vegetable dyes, and also which of the two predominates. The textile fabric is kept in the bath from a half hour to two hours, depending, as above stated, on the quality, grade and the dye stuff.

When the colors bleed freely under the action of the ingredients of the bath, and the bath becomes turbid, due to the coloring matter in suspension, a 10 per cent. solution of sodium peroxid is added, to oxidize the sus-

pended coloring matter and thus prevent its deposition on to the fabric, particularly on the whites of the material. The sodium peroxid may be added to the bath before the 60 fabric is immersed for treatment.

The caustic soda in the bath helps the sodium bisulfite to penetrate into the fabric, and therefore serves as a feeder for the sodium bisulfite. It also detaches the coloring matter from the fabric by throwing it into suspension in the bath; and, further, it attacks the fabric and thereby renders the same old looking. When it is desired to render a carpet very old looking, the 70 amount of caustic soda is increased proportionally.

After the colors in the bath have been reduced to the desired shade, the goods are taken out and washed. If the fabric treated 75 contain anilin or vegetable dyes, it will require a treatment with chlorinated water, that is, it will have to be bleached, and for this purpose a 2° Twaddell solution of chlorid of lime is preferably used. This bath 80 renders the whites of the fabric perfect, if they are not so after the treatment in the color-subduing bath.

As a rule, 80 per cent. of the textile fabrics treated by the color-subduing bath, that 85 is, the bath containing sodium hydroxid, sodium bisulfite and sodium peroxid, will come out with their whites perfect, and, therefore, will not require a treatment with chlorinated water; but, as stated, when the 90 fabric contains anilin or vegetable dyes, the additional treatment is preferable.

After the colors of the fabric have been 95 subdued by the above bath or baths, the material is thoroughly washed with soap and hot water. The soap is preferably a potassium liquid soap. This wash eliminates from the fabric all the ingredients that may have adhered thereto from the previous treatment, and it also renders the 100 textile fabric more supple. After the wash with soap, the colors of the fabric are not very brilliant, and to render the fabric and the colors brighter, or more lustrous, the fabric is washed in a slightly acid solution, 105 to acidify the colors and thereby brighten the fabric. The solution I prefer to use is acid violet, which contains 0.1 per cent. of violet.

From the above description, it will be 110 noted that the process really comprises three main steps; first, the treatment of the fab-

ric in a bath formed of reducing and oxidizing agents, the oxidizing agents predominating; when the whites of the fabric are not perfect upon leaving the above bath, it is preferably bleached with chlorinated water. The second step of the process is the thorough washing of the fabric with soap, for the purpose of eliminating the ingredients of the previous bath that may have adhered to it, and to also render the fabric more supple. The third step is the slight acidification of the fabric so as to render the colors brighter, and give to it a bluish white.

15. While I have given the relative quantities of the ingredients to be used, it must be understood that the quantities stated may be varied to an extent without materially affecting the result of the process, and therefore I do not limit myself to the exact proportions given.

I claim:

25. 1. The process of rendering textile fabrics antique which consists in subjecting the fabric to a bath formed of sodium hydroxid, sodium bisulfite and sodium peroxid until the colors of the fabric have been subdued to the desired point; then washing the fabric in a bath of chlorinated water; then washing the fabric with hot water and soap, and then passing the so treated fabric through a bath containing acid violet.
30. 2. The process of rendering textile fabrics antique which consists in subduing the colors of the fabric by a hot bath consisting of the reaction products of sodium hydroxid, sodium bisulfite and sodium peroxid;

then washing the fabric so treated, with hot water and soap to eliminate therefrom the ingredients that may have adhered to the fabric from the previous treatment; then subjecting the fabric to an acidulated bath.

3. The process of rendering textile fabrics antique which consists in subjecting the fabric to a hot bath consisting of the reaction products of reducing and oxidizing agents adapted to reduce the brightness of the colors and bleach the colors in suspension in the bath; then treating the fabric with a bleaching agent to clear the whites of the same; then washing the fabric with hot water and potassium soap, and then treating the fabric in an acidulated bluing bath.

4. The process of rendering textile fabrics antique which consists in subjecting the fabric to a hot bath of substantially 140 degrees Fahrenheit and which consists of the reaction products of caustic soda, sodium bisulfite and sodium peroxid in the proportions as specified; then treating the fabric in a bath containing chlorid of lime in the proportions specified; then washing the fabric with hot water and potassium soap, and then treating the fabric in an acidulated bath containing acid violet as specified.

In testimony whereof I have signed my name to this specification in the presence of two subscribing witnesses.

MOVSESS B. ADOM.

Witnesses:

B. JOFFE,  
PHILIP D. ROLLHAUS.